

Aug. 4, 1953

**F. R. KEMMER**

2,647,739

## METHOD FOR CALCINATION

Filed Oct. 12, 1950



INVENTOR  
*Frank R. Kemmer*

BY

*Robert Calvert*  
ATTORNEY

Patented Aug. 4, 1953

2,647,739

# UNITED STATES PATENT OFFICE

2,647,739

## METHOD FOR CALCINATION

Frank R. Kemmer, Larchmont, N. Y.

Application October 12, 1950, Serial No. 189,749

1 Claim. (Cl. 263—52)

1

This invention relates to a method and apparatus for heat treating materials in rotary kilns.

The invention is particularly useful in the calcining of Portland cement clinker and, for that reason, will be first illustrated by description in connection with such use.

The method and apparatus of the invention make possible an increase of a fifth or somewhat more in the capacity of the same kiln fired in a conventional manner and with a usual burner, produce an abnormally high and desirable temperature in the clinker at the discharge end of the kiln, shorten the combustion zone, and thus decrease the length of kiln required.

The invention provides also a method and apparatus in which powdered anthracite coal may be used as the fuel, in those regions in which anthracite is mined locally and is the least expensive fuel. The complete substitution of anthracite for such usual fuels as oil, gas, or powdered bituminous coal has not been successful heretofore in cement manufacture; the low content of volatile matter and the high percentage of fixed carbon in anthracite coal retard the combustion of this coal when it is tried as the powdered fuel in a cement kiln. As a result, the flame is not of the usual plume shape but is considerably longer. The long flame gives more wide distribution of the heat and less concentration of it where desired in the firing end of the kiln. The limit to the amount of anthracite that may be substituted has been around 50% of the total weight of coal used in the firing process.

Briefly stated, the invention comprises a burner for an aeriform suspension of a fluid fuel or powdered coal, the burner having a slit orifice serving to shape the flame of the burning fuel into a flat band, and means for approximately parallelizing the band flame, both angularly and longitudinally, with the surface of the charge in the kiln. In the preferred embodiment, the invention includes also means for directing a stream of secondary air, for the combustion of the fuel, between the band flame and the cement or other material being heated. This apparatus in operation gives a band flame in close proximity to the exposed surface of the charge and approximately parallel thereto.

The invention comprises, also, the method of heat treating material with the spaced band or ribbon flame as described herein.

The invention will be further illustrated by description in connection with the attached drawings to which reference is made.

Fig. 1 shows a side sectional view of the firing 55 of the kiln firing end described are those which

2

end of a rotary kiln constructed in accordance with the invention.

Fig. 2 is a sectional view on line 2—2 of Fig. 1.

Fig. 3 is a sectional view on line 3—3 of Fig. 1.

Fig. 4 is a sectional view on line 4—4 of Fig. 1.

The sectional views are in the direction of the arrows on the respective section lines. The figures are in part diagrammatic. The parts not illustrated are conventional.

There are shown an inclined rotary kiln with outer shell 10 driven by conventional ring gear 12 and gear wheel 14, the charge 16 undergoing heat treatment, and a layer 18 of the material of the charge caked upon the refractory lining 20 inside the shell of the kiln.

The burner 22 has a discharge end 24 in the shape of a slit. The slit is angularly inclined, as shown in Fig. 2, so that the flame 26 is approximately parallel to the exposed surface of the material 16 being heat treated. While the flame 26 spreads and becomes irregular, it retains the general form of a ribbon or band.

Secondary air is admitted through the duct 28 and drawn upward by the natural draft of the system. A deflecting baffle 30 extends across the wall 32 of the duct and deflects the stream of secondary air, to the right in Fig. 1, that is, under and into the band flame 26. This direction of the secondary air prevents the band flame from striking down for any substantial period of time upon the material being heated. This direction of the secondary air also promotes prompt combustion of the fuel.

Another deflector 31 is mounted on the side wall of the hood or firing head. It may be a part 35 of the ceramic or cement construction of the head as shown, for instance, in Fig. 2. The location of this second deflector is adjacent to the end of the kiln and on the up-side thereof as the kiln is rotated. The position is below the level of the upper edge of the band flame. This deflector extends in a sloping manner generally toward this upper edge of the flame. This deflector 31 serves the purpose of tilting the stream of secondary air, so as to cause its upper surface to parallel more closely the angle of the band flame.

In case of cement manufacture, this secondary air ordinarily is that which issues from the clinker cooler disposed below the rotary kiln. In a representative run with the apparatus described, the temperature of the secondary air delivered from the cooler to the kiln was 819° F., as compared to only 692° for the same setup with standard round burner and plume flame.

Materials of construction for the various parts

are usual in apparatus of this kind. Thus, the shell 10 in the kiln may be steel, the lining 20 a high grade refractory block, the duct 28 fire brick, the burner 22 with the slit opening 24 steel, and the deflector 30 fire clay in fired condition.

Some of the principal advantages of the invention are stated above. There are others.

What is desired in the calcination of cement or the like is intense heat transfer by radiation. The equipment shown in Figs. 1 and 2, for instance, keeps the flame out of contact with the said material and in the quadrant or quarter of the kiln containing material 16. The flame is in extremely close juxtaposition to the material, however, so that the radiation to the material is much greater for unit area of exposed surface thereof than to the more remote parts of the circumference of the kiln. There is obtained not only increased transfer of heat to the material to be calcined, with proportionate attendant increase in the rate at which the material may be fed through the kiln, but also a decreased percentage of the total heat lost through the kiln wall.

As a result of lesser heating of the kiln lining, there is a decrease in the thickness of the caked layer 18 inside the kiln, as from the usual 8 or 9 inches to about 5 to 6 inches. This increases the effective free space within the kiln.

Using this system in Portland cement manufacture, there is possible an increase of production per kiln in excess of 18% of the normal production capacity. To obtain this increase of capacity, without decrease of the final temperature of calcination below the usual, the speed of rotation of the kiln is increased.

With the apparatus and method described, the firing zone in the cement kiln may be shortened from the usual 25-30 feet to 15-20 feet.

The operation of the equipment and the method will be evident from the discussion that has been given above.

In general, the kiln is mounted at a slight inclination downward towards the discharge end and rotated in a usual manner. The fuel if oil is atomized or if coal is suspended in finely powdered form in the barrel of the burner 22. The atomizing or suspending medium is air. The atomized oil or the aeroform suspension of the coal is then delivered through the slit 24 constituting the firing or discharge end of the burner. Natural gas may be used as the fuel, with all the air for its combustion introduced outside the stream of the gas issuing from the slit in the burner.

The burner is mounted by usual means, as by bolts securing it to a supporting framework (not shown) at such an angle radially that the length of the slit 24 is approximately parallel to the exposed surface of the material being calcined. This gives a flame that at the start is also approximately parallel to the said surface, all as shown in Figs. 2 and 4. In the case of cement clinker this angle of repose in the rotating kiln is about as shown in Fig. 2. The angle varies somewhat and reaches about the angle shown by the steeper line 17 before sliding or tumbling down to the zone 16. In addition to the angular mounting of the burner radially in the manner stated, the mounting means also establish the longitudinal axis of the burner approximately in the same slope as the slope of the rotary kiln itself. The means are usual, the setting being merely adjusted to give the longitudinal parallelizing. This parallelizing of the burner and the

band shaped flame issuing from the burner prevent the flame, as it extends into the kiln, from striking down on the material being calcined and the stream of secondary air under the flame furnishes additional protection against overheating; the invention includes not only the parallelizing of the burner and the band flame with the kiln, as stated, but also the discovery that striking of the flame at a sharp angle upon the material being calcined is objectionable and in fact is not permissible, particularly when there is used a fuel of such great calorific power as powdered anthracite coal.

With the condition described, it is now possible to substitute powdered anthracite to the extent of 100% for bituminous coal or oil.

It is possible under my conditions also to form quickly the coating 18 in the firing end of the kiln. This quick formation of the coating is contrary to experience with the conventional plume flame of a cylindrical burner. With the conventional burner and flame, there is considerable lapse of time after a kiln has been rebricked and placed under fire before the coating 18 forms. The building of a satisfactory coating to a thickness of 1 to 2 inches may require as long as twelve to twenty-four hours. With my method and apparatus, on the other hand, I form the initial coating and build it up to this thickness within about two hours.

The dimensions of the burner will be varied in accordance with the size of the kiln being fired, the temperature required, and the rate of passage through the kiln of the material to be calcined. In general, the size of the slit is one which has approximately the same area as the conventional round outlet of the usual type of oil or powdered coal burner. We have found particularly satisfactory results when the length of the burner slit is about ten to ninety times the width of the slit. With coal, dimensions that are suitable for the outlet slit in the burner are lengths of 3 to 6 feet and widths of  $\frac{3}{4}$  to 2 inches or so. The length of the burner slit will be larger, the larger the kiln diameter. Three feet is about the right length of slit for a 9 foot kiln and five feet for a 12 foot kiln.

In general, the length of the slit in the burner is about 30% to 40% of the overall diameter of the kiln; that is of the shell 10, or about 20% to 30% less than the width of the exposed surface of the charge being calcined and represented by 16 in the drawings.

The spacing of the burner is about 4 to 10 inches above the level of the upper surface of material 16.

The invention will be further illustrated by the specific example of the practice of it.

#### Example

I have applied my method and apparatus to a rotating kiln having a steel shell 9 feet in diameter by 125 feet long, with a lining of refractory 6 inches thick, with a conventional burner of a diameter of 8 inches, and with powdered bituminous coal as the fuel. The ordinary plume-like flame made possible an output of clinker averaging 39 barrels per hour. With my slit burner, of length of slit approximately 3 feet and width  $1\frac{1}{2}$  inch, I increased the output to an average of 46.2 barrels of cement clinker per hour, a gain of 18% in rate of production.

My method and apparatus also give other advantages over the conventional burner and method. Thus the flame temperature was raised

by approximately 43° F. to 2746° F., with the possibility of maintaining a flame temperature of 3000° F. if desired. The temperature of clinker discharge from the kiln was 2170° F. as compared to 2040° F. in the conventional operation. The temperature to which the secondary air was pre-heated in the clinker cooler was 760° F. as compared to 600° F. with the usual round burner. In a series of separate kilns in which my method and apparatus were used, it was found in each instance that the speed of the kiln could be increased. In fact, the speed was increased. Also the speed of the clinker cooler was increased, to take away the clinker and prevent accumulation of the increased production to an undesirable depth in the bed in the cooler. The proportion of total heat supplied which goes into the finished product was increased, with resulting fuel economy per barrel of cement made.

The procedure of the example and the general method described is useful also in calcining limestone to lime, aluminum hydrate to alumina, magnesite to magnesia for basic refractories, sintering red mud from bauxite refining by the Bayer process, nodulizing ores of iron or manganese, and volatilizing zinc oxide from zinc plant residues.

So used, my method and apparatus give increased capacity per kiln and fuel economy per ton of output. Also there may be used anthracite to the extent of 75% or so, the remainder being oil or bituminous coal. For some uses, anthracite may be employed exclusively.

When the material is changed from the Portland cement of the example, the temperature established in the material is made that which is accepted practice for the particular material used. The rate of feed and consequently the rate of production per kiln is increased, however,

to make full use of the greater rate of heat transfer from the closely spaced wide band of flame to the material being processed.

It will be understood that it is intended to cover all changes and modifications of the examples of the invention herein chosen for the purpose of illustration which do not constitute departure from the spirit and scope of the invention.

What is claimed is:

The method of heat treating material in an inclined rotary kiln which comprises advancing the material with inclined exposed surface through the kiln by rotation thereof, introducing into the lower quadrant of the firing end of the kiln, which quadrant contains the material to be treated, a flame that extends generally parallel to the length of the kiln, that is of the general shape of a band, that is disposed in close proximity to the inclined surface of the said material, and that is tilted so that the flame is approximately parallel to the angle of repose of the said material, and introducing and deflecting a protective stream of air between the said band and material, so that the stream is guided into a path that is approximately parallel to the flame and surface of the said material, the introduction of the air serving to prevent contact of the flame with the material.

FRANK R. KEMMER.

References Cited in the file of this patent

UNITED STATES PATENTS

| Number    | Name     | Date          |
|-----------|----------|---------------|
| 2,034,180 | Glenn    | Mar. 17, 1936 |
| 2,487,369 | Plotner  | Nov. 8, 1949  |
| 2,555,289 | Nagel    | May 29, 1951  |
| 2,584,808 | Newhouse | Feb. 5, 1952  |